

Sept. 27, 1960

N. DRISCH ET AL  
PROCESS OF PRODUCING A SHRINKABLE  
CELLULOSE TEXTILE FILAMENT  
Filed Dec. 14, 1956

2,954,270



INVENTORS  
NICHOLAS DRISCH  
PIERRE SCHNELLER  
BY  
*Chleek*  
ATTORNEY

1

2,954,270

## PROCESS OF PRODUCING A SHRINKABLE CELLULOSE TEXTILE FILAMENT

Nicolas Drisch and Pierre Schneller, Paris, France, assignors to Chimiotex Societe Anonyme, Tangier, North Africa, a corporation of Tangier

Filed Dec. 14, 1956, Ser. No. 628,217

Claims priority, application France Dec. 14, 1955

## 1 Claim. (Cl. 18—54)

This invention relates to a method for producing high bulk yarns composed of a mixture of shrinkable and non-shrinkable fibers, and has for an object to provide novel and improved methods for producing fibers for use in such yarns.

According to the present invention, new high-bulk yarns are obtained by a treatment in a very hot aqueous medium without tension, of yarns containing on the one hand shrink-proof fibers and on the other artificial cellulosic fibers having high shrinkage under these conditions.

More specifically, these yarns are obtained by association of a sliver of shrink-proof filaments and of a continuous sliver of shrinkable artificial cellulose filaments with high elongation.

The continuous shrink-proof filaments may be cellulosic filaments having very high tenacity and low elongation, which are obtained by the process described in French Patent No. 985,847 (U.S. Patent No. 2,586,796). Continuous filaments having very high elongation, which are more particularly suitable for use in the new yarns according to the invention, may be obtained by the viscose process with the application of various measures, in any desired combination.

(a) Spinning is carried out at low speeds, for example from 15 meters to 30 meters per minute. This speed may, however, be increased up to from 70 meters to 120 meters per minute by employing a tube aligned with the spinneret described in French Patent No. 1,006,078, dated November 10, 1947 (U.S. Patent No. 2,511,699, dated June 13, 1950).

(b) Spinning in a single coagulating bath, containing about 115 grams per liter of sulphuric acid; 250 grams per liter of sodium sulphate; and 120 grams per liter of zinc sulphate. At the higher spinning speeds the acidity should be slightly increased, for example to 120 grams to 125 grams per liter of sulphuric acid and the zinc sulphate should be increased for example to 125 grams to 130 grams per liter. A viscose having a high sodium chloride salt point of more than 14 and preferably more than 16, as determined in accordance with the procedure set forth in the Brandenberger Patent No. 1,544,631, should be used.

(c) Reduced drawing at spinning, just sufficient to produce an appropriately organized and oriented filament (10% to 25%). This drawing should not exceed about 20%, while the filaments preferably subsequently undergo, in a second dilute bath at 85° C. at least, a high drawing of at least 30%.

(d) Addition to the viscose and/or to the bath of agents giving rise to the formation of thick-skinned filaments, such as amines or polyglycol ethers.

(e) The final drawing, after wet finishing, or even after dry finishing of the purified filament, can reach 60% of the elongation at break. Wet drawing is carried out in all cases, and it is essential to dry under tension without any possibility of shrinkage.

The most important conditions are (a), (c) and (e), and it has been possible to obtain, for example, with a

2

normal viscose spun at 25 meters per minute, with 20% drawing during spinning, a yarn having an elongation of 45%, which may be 20% in the wet state, and which is thereafter dried under tension to give a yarn which shrinks by 20% to 25% in a boiling water bath.

The drawing is a flow sheet illustrating the preferred embodiment of the invention.

The invention will be better understood by referring to the examples and the claims attached hereto.

10

## Example 1

A sliver of 3300 denier/1440 filaments having very high elongation as in the foregoing is doubled with a sliver of 3300 denier/8000 filaments of regenerated cellulose having a dry tenacity of 6.8 grams with an elongation of 9.5%, and the double sliver is subjected to drawing to breaking point on the device described in U.S. Patent No. 2,746,091, for a device for the manufacture of mixed yarns, whereafter the broken yarn is drawn and twisted in such manner as to form a No. 90 yarn (French) which is wound on cops. This yarn has a shrinkage of 25% in boiling water and thus acquires high bulk.

## Example 2

25 There are prepared yarns having a moist elongation of 45% obtained by spinning at a salt point of 15 a viscose, containing 2% of thiodiglycol (according to French Patent No. 1,111,580, dated September 3, 1954; U.S. Serial No. 532,799, filed September 6, 1955, now Patent No. 2,912,299) with a drawing at spinning of 20%. This sliver is then drawn by 18% and dried under tension. The shrinkage on wetting of the fiber obtained is then 23%.

35 This fiber cut to 100 millimeters is mixed in a proportion of 50% with a fiber spun under similar conditions, the drawing of which during spinning was 120%. This fiber has been freely dried and the shrinkage in boiling water was only 1%.

40 The mixture of the two fibers is worked on conventional equipment for carded wool, and a No. 40 yarn (metric) is formed with a twist of 400 turns. This yarn is woven in twill weave and this fabric is then dyed with the aid of a mordant. During the dyeing, a shrinkage of 35% occurs in each dimension. The apparent bulk of the yarn is about twice that of the initial yarn.

45 The fabric thus obtained only requires a finishing treatment with 5% of ureaformaldehyde. The finished fabric is completely crease-resistant and shrink-proof in washing, and has the characteristics of a woolen fabric.

## Example 3

50 Same example as before, but the shrinkable yarn is mixed with 50% of a normal acetate fiber.

55 The fabric obtained is crease-proof and shrink-proof without any further treatment.

## Example 4

56 A viscose containing 9% of cellulose and 6% of caustic soda, prepared with the aid of 50% carbon disulphide, calculated on the alpha cellulose and containing 0.15 millimol of waxy polyhydroxyethylene to 100 grams of alpha cellulose, is spun at a salt point of 16.5 into a bath containing 120 grams of sulphuric acid, 231 grams of sodium sulphate and 128 grams of zinc sulphate per liter. The bath is at 48° C. and the viscose is preheated to this temperature immediately on the upstream side of the spinneret.

57 The spinning device comprising a tube as described in French Patent No. 1,066,078 (U.S. Patent No. 2,511,699) referred to above is employed. On leaving the spinning bath, the yarn passes over a first feed roller, which effects a 12% drawing of the yarn in relation to the

speed of the viscose in the spinneret holes. The yarn then passes into a second 1% sulphuric acid bath heated at 89° C., and is taken up on leaving this bath by a second feed roller running at a tangential velocity 30% higher than that of the first feed roller. It is then wound at the same or a slightly higher speed onto a rigid bobbin, the linear winding speed being of the order of 75 meters per minute.

After winding to a sufficient depth of yarn on the bobbin, the wound mass is washed on the bobbin and then desulphurized with a hot dilute alkaline bath and, if desired, bleached and boiled.

The yarn is then unwound and again drawn by 18%, whereafter it is wound on another rigid bobbin, on which it is subjected to drying.

The dried yarn has a tenacity of 3.5 grams in the dry state and 2.5 grams in the wet state, with an elongation at break of 12% in the dry state and 17% in the wet state. On wetting followed by drying without tension, it is capable of a shrinkage of 30%.

*Example 5*

A group of 10,000 filaments is spun and continuously treated, whereafter it is passed over a member permitting of the most complete possible relaxation and is again continuously hot-drawn, the drawing being 70% of the elongation at break in the wet state, that is to say, 40% in the example chosen. The group of filaments is then dried on heated rollers without any possibility of shrinkage.

In both cases, the group of filaments obtained can be cut into sections or converted into a tow of discontinuous fibers on a machine of the "converter" type or by drawing to breaking point on a stapling frame.

5

4

It is obvious that the invention is in no way limited to the specific examples described, but also includes any modifications in the same spirit. It should be emphasized that the shrinkage is not necessarily produced on the mixed yarns. It is advantageously produced on articles woven or knitted with said yarns for the purpose of producing swelling effects and a softer handle.

What is claimed is:

The process of producing a shrinkable cellulosic textile filament, which comprises spinning into a bath having an acidity of 125 grams to 130 grams sulphuric acid per liter and a zinc sulphate content of 125 grams to 130 grams per liter having a temperature of about 48° C. in the presence of a polyglycol modifying agent which delays coagulation, viscose having a sodium chloride salt point greater than 14 and preheated to the temperature of the bath at a rate of 70 meters to 120 meters per minute through a confined zone with less than 20% drawing during the spinning, drawing the spun filaments in a bath having a temperature of 85° C. to 89° C. to an elongation in excess of 30% washing and finishing drawing said finished filaments in an additional stage by about 18% and drying under conditions to prevent shrinkage.

25

30

References Cited in the file of this patent

UNITED STATES PATENTS

|           |          |       |                |
|-----------|----------|-------|----------------|
| 2,369,190 | Thurmond | ----- | Feb. 13, 1945  |
| 2,511,699 | Drisch   | ----- | June 13, 1950  |
| 2,535,044 | Cox      | ----- | Dec. 26, 1950  |
| 2,696,423 | Dietrich | ----- | Dec. 7, 1954   |
| 2,852,333 | Cox      | ----- | Sept. 16, 1958 |